

April 15, 1941.

L. D. MANNES ET AL

2,238,495

METHOD OF COLOR PHOTOGRAPHY

Filed April 12, 1940

FIG. 1



FIG. 2



FIG. 3



LEOPOLD D. MANNES  
LEOPOLD GODOWSKY JR.  
INVENTORS

BY *Newton M. Perini*  
*R. Frank Smith*  
ATTORNEYS

## UNITED STATES PATENT OFFICE

2,238,495

## METHOD OF COLOR PHOTOGRAPHY

Leopold D. Mannes, New York, N. Y., and Leopold Godowsky, Jr., Westport, Conn., assignors to Eastman Kodak Company, Rochester, N. Y., a corporation of New Jersey

Application April 12, 1940, Serial No. 329,344  
In Great Britain May 10, 1939

6 Claims. (Cl. 95—2)

This invention relates to an improved method of color photography and includes a method of producing sensitive photographic elements, color photographic elements themselves and methods of processing photographic elements.

It is known that colored photographic images may be formed by using a developing agent which forms a colored compound on development of a silver salt. The colored compound thus formed is deposited adjacent the silver grains of the silver image during the development. It is also known that a colored image may be formed by adding to certain developer solutions or by incorporating in the photographic silver halide emulsion before or after exposure a compound which couples, during development, with the oxidation product of the developing agent, and forms a coloring substance which is likewise deposited adjacent the silver grains of the silver image during development. Such a compound, which is employed in conjunction with a developing agent for the silver and which couples with the oxidation product thereof during development, is referred to herein as a color coupler.

It is known that when color couplers are incorporated in the photographic emulsions themselves difficulties arise through the fact that these color formers tend to wander from the emulsion in which they are incorporated during the coating of the emulsions on a support and during processing operations, in which the emulsions are treated with liquid baths such as developing baths and fixing baths. Many proposals have been made which have had for their object to prevent or retard the wandering of the color couplers, e. g. by employing couplers containing in the molecule group intended to render the color couplers non-wandering.

It has now been found that the color couplers show very much less tendency to wander in acid solutions than in alkaline solutions and that if the emulsions containing them are so prepared, coated and processed that they are never subjected to liquid baths other than those which are of an acid character until the coupling development has taken place, those color couplers which will diffuse under alkaline conditions can, nevertheless, be used without undue diffusion taking place.

According to one feature of the present invention, the method of producing a sensitive photographic element in which a colored image can be produced by development of a silver salt therein consists in incorporating a color coupler in a gelatino-silver salt emulsion and coating such

emulsion on a support while maintaining the pH of such emulsion on the acid side of neutrality during such incorporation and such coating.

In the accompanying drawing, Fig. 1 is a sectional view of a single layer photographic element made according to our invention, Fig. 2 is a sectional view of a multi-layer photographic element made according to our invention and Fig. 3 is a view, partly in section, of apparatus used in the treatment of film according to our invention.

The invention particularly includes the method of producing a multi-layer sensitive color-photographic element by coating a plurality of gelatino-silver salt emulsion layers on a single support in which a color coupler is incorporated in at least one of the emulsions before coating and the pH of such emulsion is maintained on the acid side of neutrality during such incorporation and such coating.

Preferably, the emulsion is maintained at a pH below 6.5, more particularly, below 5.5 during such incorporation and coating.

The invention also includes a color photographic element having a support 10 and at least one layer 11 coated on such support (Fig. 1), which layer consists of a gelatino-silver salt emulsion in which a color coupler has been incorporated while maintaining the pH of the emulsion on the acid side of neutrality during the incorporation of the color coupler and coating on the support.

More particularly, the invention includes a multi-layer color photographic element in which two or more emulsion layers are inseparably coated on a single support 10 (Fig. 2) each consisting of a gelatino-silver salt emulsion in which a color coupler has been incorporated while maintaining the pH of the emulsion on the acid side of neutrality during the incorporation of the color coupler and coating on the support. Such multi-layer color photographic element may have three emulsion layers 12, 13 and 14 respectively sensitized to blue, red and green regions of the spectrum. The element may include the usual yellow filter layer 15 between emulsion layers 13 and 14. The invention also includes the method of processing a photograph element consisting of a support having coated thereon at least one silver salt emulsion layer containing a color coupler in which any processing baths to which the element is subjected which are not intended to bring about reaction of the color coupler are maintained on the acid side of neutrality, and development with a color-forming developer is

carried out without immersion of the element in an alkaline liquid.

The development with a color-forming developer may be carried out by causing the emulsion layer or layers which contains or contain the color coupler to imbibe a color-forming developer of acid reaction and then treating it or them with the alkali necessary for development and coupling without immersion in liquid. Such treatment with alkali can be effected conveniently by bringing the moist and swollen emulsion into contact with ammonia gas. The three differentially-color sensitized layers may or may not be separated by gelatine intermediate layers. The emulsion may be silver bromide or silver chloride, or some may be of silver chloride and some of silver bromide. Thus, the two lower layers may be silver chloride emulsions and the upper layer a silver bromide emulsion, the choice of the material depending upon whether the element is to be used for camera exposure or printing.

The color couplers are incorporated in the layers before coating by mixing them with the respective emulsions while maintaining such emulsions at a low pH, i. e. on the acid side of neutrality and preferably below 6.5, most desirably below 5.5. The color couplers may be any of the color formers known and described in the literature, e. g. phenols, naphthols, compounds containing a reactive methylene group such as acetoacetic esters, pyrazolones, arylacetonitriles and the like. Examples of suitable color couplers (also called "coupling components") are acetoacetanilide,  $\beta$ -naphthoyl acetonitrile, and  $\alpha$ -hydroxy diphenyl.

At no time during the incorporation of the color coupler in the emulsion or during the coating of the emulsion should the pH be allowed to or above the point of neutrality.

In the case of a film, for example a motion picture film 16 (Fig. 3) which contains the color couplers in three differentially color-sensitized layers on the same side of the support, the film may be processed to a negative by bathing it for a short time in an acid solution of a color developer, for example one of the following formula:

|                                     |       |        |    |    |
|-------------------------------------|-------|--------|----|----|
| Diethyl paraphenylenediamine hydro- |       |        |    |    |
| chloride                            | ----- | gms.   | 20 |    |
| Sodium bisulphite                   | ----- | do     | 10 |    |
| Potassium bromide                   | ----- | do     | 2  |    |
| Water to make                       | ----- | liters | 1  | 50 |

In the treatment of a chloride emulsion, the quantity of potassium bromide may be decreased, or this may be replaced by a soluble chloride. The film 16 is immersed in this acid solution of color developer 18 in tank 17 just long enough to wet it thoroughly, a time of one minute being usually sufficient. After immersion the excess of liquid is removed, e. g. by a squeegee 22.

The film is then brought into contact with ammonia gas in chamber 19 for a sufficient time to render it thoroughly alkaline. This causes development to take place whereby the latent images are developed to silver and simultaneously the color coupler couples with the oxidation product of the developing agent. A few minutes' exposure to ammonia gas is sufficient to cause development to take place, 5 minutes being adequate in the majority of cases. The ammonia gas is passed through tank 19 by means of pipes 20 and 21.

After development has taken place the film is washed in a liquid of sufficiently low pH value to arrest further color development. A weak sodium bisulphite solution having a pH between 75

about 4 and 5 is generally suitable for this. The silver and residual silver halide can then be removed by treatment in a bath containing ferricyanide and hypo, leaving clear, transparent negative dye images.

If it is desired to process the film to a positive, the latent images can first be developed with an acid non-coupling developer, such as an acid amidol or acid ferrous oxalate developer. After washing and resensitizing (if necessary) the film is exposed to light to render the residual silver halide developable. The development of the residual silver halide is then carried out by imbibition of an acid color developer and treatment with ammonia gas as described above.

Instead of using ammonia gas alone, a mixture of ammonia and sulphur dioxide, or of ammonia and carbon dioxide, may be used. In such cases, either ammonium sulphite or ammonium carbonate is formed in the film which may give in some cases more desirable development conditions.

It will be seen that in the above processing the emulsions are not allowed to come into contact with any liquid baths whose pH values are on the alkaline side of neutrality until the time when color development actually takes place. Moreover, the development is carried out under such conditions that little molecular diffusion of the developer can take place, but this is permitted to act in the medium of swollen gelatine.

The film treated may carry a sound track which may be processed to minus-red color by recording it in the layer which contains a color-coupler for minus-red and by developing the image in the sound track area alone by means of a coupling developer applied by an applicator roller. The processing of the sound track may proceed any other step in the processing since the acidity of the first developing solution applied for development of the picture areas will arrest further action of the minus-red color coupler.

We claim:

1. The method of forming a colored image in a photographic silver halide layer, which comprises incorporating in the layer at a pH lower than about 6.5 a compound which couples with an aromatic amino developing agent in alkaline solution to form a dye, and which diffuses from the layer in alkaline solution, exposing the layer to light to which it is sensitive, immersing the exposed layer in an acid solution of an aromatic amino developing agent, and then subjecting the layer for a short time to alkaline vapors to form a colored image in the layer.

2. The method of forming a colored image in a photographic silver halide layer, which comprises incorporating in the layer at a pH lower than about 6.5 a compound which couples with an aromatic amino developing agent in alkaline solution to form a dye, and which diffuses from the layer in alkaline solution, exposing the layer to light to which it is sensitive, immersing the exposed layer in an acid solution of an aromatic amino developing agent, and then subjecting the layer for a short time to ammonia vapors to form a colored image in the layer.

3. The method of forming a colored image in a photographic silver halide layer, which comprises incorporating in the layer at a pH lower than about 6.5 a compound which couples with an aromatic amino developing agent in alkaline solution to form a dye, and which diffuses from the layer in alkaline solution, exposing the layer to light to which it is sensitive, immersing the

exposed layer in an acid solution of an aromatic amino developing agent, for about one minute, and then subjecting the layer for about five minutes to ammonia vapors to form a colored image in the layer.

4. The method of forming a multi-color image in photographic silver halide layers, which comprises incorporating in three superposed layers each sensitive to a different region of the visible spectrum, at a pH lower than about 6.5, three different color couplers which couple with an aromatic amino developing agent in alkaline solution to form dyes and which diffuse from the layers in alkaline solutions, exposing the layers to light to which they are sensitive, immersing the layers in an acid solution of an aromatic amino developing agent, and then subjecting the layers for a short time to the action of alkaline vapors to form colored images in the layers.

5. The method of forming a multi-color image in photographic silver halide layers, which comprises incorporating in three superposed layers sensitive respectively to the blue, green, and red regions of the visible spectrum, at a pH lower than about 6.5, color couplers, forming yellow, magenta, and blue-green dyes, respectively, which couple with an aromatic amino developing agent in alkaline solution to form dyes and which

diffuse from the layers in alkaline solutions, exposing the layers to light to which they are sensitive, immersing the layers in an acid solution of an aromatic amino developing agent, and then subjecting the layers for a short time to the action of alkaline vapors to form colored images in the layers.

6. The method of forming a multi-color image in photographic silver halide layers, which comprises incorporating in three superposed layers sensitive respectively to the blue, green, and red regions of the visible spectrum, at a pH lower than about 6.5, color couplers, forming yellow, magenta, and blue-green dyes, respectively, which couple with an aromatic amino developing agent in alkaline solution to form dyes and which diffuse from the layers in alkaline solutions, exposing the layers to light to which they are sensitive, immersing the layers in an acid solution of an aromatic amino developing agent, and then subjecting the layers for a short time to the action of alkaline vapors to form colored images in the layers, and thereafter arresting further color development by immersing the layers in an acid bath.

LEOPOLD D. MANNES.  
LEOPOLD GODOWSKY, JR.